

# UNITED STATES PATENT OFFICE.

HERBERT PASCHKE, OF NEW YORK, N. Y.

## ART OF PRODUCING MASTIC.

No. 832,697.

Specification of Letters Patent.

Patented Oct. 9, 1906.

Application filed October 6, 1904. Serial No. 227,505.

*To all whom it may concern:*

Be it known that I, HERBERT PASCHKE, a citizen of the United States, and a resident of the city of New York, borough of Manhattan, 5 in the county of New York and State of New York, have invented a new and Improved Art of Producing Mastic, of which the following is a full, clear, and exact description.

This invention relates to the bituminous mastics formed and capable of employment in a cold state and without the application of heat of any sort, so that the article may be produced as expeditiously as common mortar and applied in essentially the same manner.

The invention possesses not only the advantage of eliminating the use of heat in all forms, but also that of an entirely waterproof composition, especially useful where 20 waterproof walls, floors, ceilings, or analogous structures are to be produced.

In order that my invention may be fully understood, I will now proceed to describe, as an example, the preferable manner of practicing the same.

In order to produce a cold waterproof mastic, I employ a pulverized or finely-divided cold (and therefore set) soluble bituminous or other equivalent substance. The degree 30 to which this substance is pulverized or divided may be varied and depends much upon the nature of the work to be performed. It may be stated, for example, that for work such as the production of mastic for laying 35 ordinary brick the bituminous or equivalent material should be pulverized to grains of approximately one-sixteenth ( $\frac{1}{16}$ ) of an inch in diameter. I next take a solvent of the said bituminous or other equivalent substance. 40 In the case of a bituminous substance, such as asphalt, I prefer to employ as a solvent benzim or naphtha. This solvent is preferably utilized by first mixing it with a relatively small quantity of the bituminous or 45 equivalent substance, forming a semiliquid or viscous solution, which is applied to the pulverized bituminous material forming the base, so as to convert the whole into a stiff plastic mass, which assumes this form with- 50 out the employment of heat of any sort and which may be employed as a substitute for mortar and cement in forming walls, coverings, or for laying brick, tile, or stone in practically the same manner that ordinary mor- 55 tar and cement are employed.

The pulverization of the bituminous or

other material forming the base of the mastic is important in my invention, since with the material pulverized, as explained, upon the application of the solvent the solvent at- 60 tacks the outer surface of each grain of the said material forming the base and softens said outer surface, causing the grains to adhere strongly together without, however, running the compound into a homogeneous 65 or uniform mass, the interior portions of the grains of the bituminous material remaining for the time unaffected, so that the material retains to some extent its solid proportions, thus imparting to the mastic a stiffness 70 which enables it to be utilized in the manner explained. The mastic should be utilized immediately after it is formed and before the action of the solvent has brought about uniform or complete dissolution of the bitumi- 75 nous or equivalent material. After the mastic has been laid on brick, stone, tile, or whatever desired the action of the solvent goes on, and finally the grains of pulverized material are wholly dissolved and run one 80 into the other, so that a uniform solid mass is produced. Evaporation of the solvent goes on and the mastic begins to take its permanent or set form, not in the shape of granulated or pulverized material, however, but in 85 the shape of a concrete uniform mass, the previously plastic condition of which enables it to be worked and set exactly as desired. In securing the result before described it will be understood that the solvent is in such 90 quantity in proportion to the mass of material as to ultimately dissolve the entire mass, as before described, and I find in practice that good results are ordinarily secured by the use of about six or seven gallons of sol- 95 vent to each one hundred pounds of the mass of granulated asphaltic material. The practice above explained of utilizing as a solvent a viscous or semiliquid compound composed partly of the solvent and partly of a quantity 100 of the bituminous material constituting the base of the mastic is also of much importance in this invention. In doing this a certain quantity of the bituminous material is combined with the raw solvent, so as to form the 105 viscous or semifluid solution referred to, and this solution is poured upon the pulverized granular mass forming the base of the mastic. The result is that the bituminous material first compounded with the solvent 110 holds the solvent in a sort of suspension and retards its evaporation sufficiently to allow

it to have the necessary action upon the pulverized bituminous material before the solvent evaporates. Were the raw solvent applied to the pulverized mastic the tendency 5 would be for the solvent rapidly to evaporate and for this evaporation to become complete before the solution of the bituminous or other material is completed, thus defeating, partly at least, the purpose of the invention. In 10 special cases, however—such, for instance, as those in which but small quantities of the mastic are produced at an operation and the mastic thus produced instantly employed—it is possible to employ a raw solvent mixed directly with the pulverized bituminous material. With this mastic a certain quantity of inert material—such as sand, quartz, or the like—may be used or not, as desired, without in any way departing from the principle of 15 my invention.

Having thus described the preferred manner of practicing my invention, I claim as new, and desire to secure by Letters Patent—

1. The improvement in the art of producing a cold, waterproof mastic, which consists, first, in pulverizing or granulating a cold soluble waterproof substance, and, second, in subjecting the said granulated waterproof substance to the action of a solution 25 composed of a soluble waterproof material and a volatile solvent of the same, whereby the evaporation of the solvent is delayed sufficiently to enable it to attack the outer surfaces of the said grains of waterproof material, softening said surfaces and causing said grains to adhere together and form a stiff 30 plastic mass.

2. The improvement in the art of producing a cold, waterproof mastic, which consists, first, in pulverizing or granulating a cold bituminous material, and, second, in subjecting said granulated bituminous material to the action of a solution composed of a bituminous material and a volatile solvent of 40 the same, whereby the evaporation of the solvent is delayed sufficiently to enable it to attack the outer surfaces of the said grains of bituminous material, softening said surfaces and causing said grains to adhere and form 45 a stiff plastic mass.

3. The improvement in the art of producing a waterproof structure, which consists, first, in pulverizing or granulating a cold soluble waterproof material, second, in causing 55 a solvent sufficient in quantity to ultimately dissolve the entire mass to attack the outer surfaces of the grains of said cold granulated material and softening the same whereby the grains adhere to each other and form a stiff 60 plastic mass without the utilization of heat, and, third, in laying said stiff plastic mass in

the desired form or position before the action of the said solvent extends to and dissolves the interior parts of said grains of cold granulated material.

4. The improvement in the art of producing a waterproof structure, which consists, first, in pulverizing or granulating a cold bituminous material, second, in causing a solvent sufficient in quantity to ultimately dissolve the entire mass to attack the outer surfaces of said grains of cold bituminous material and softening the same, whereby the grains adhere to each other and form a stiff plastic mass without the utilization of heat, 70 and third, in laying said stiff plastic mass in the desired form or position before the action of the solvent extends to and dissolves the interior parts of said grains of bituminous material.

5. The improvement in the art of producing a waterproof structure, which consists, first, in pulverizing or granulating a cold soluble waterproof material, second, in subjecting said granulated waterproof material to the action of a solution composed of a soluble waterproof material and a volatile solvent of the same, whereby the evaporation of the solvent is delayed sufficiently to enable it to attack the outer surfaces of the said grains of waterproof material, softening said surfaces and causing said grains to adhere and form a stiff plastic mass, and, third, in laying said plastic mass in the desired form or position before the action of the said solvent extends to 90 and dissolves the interior parts of said grains of soluble waterproof material.

6. The improvement in the art of producing a waterproof structure, which consists, first, in pulverizing or granulating a cold, bituminous substance, second, in subjecting said granulated and bituminous substance to the action of a solution composed of a bituminous material and a volatile solvent of the same whereby the evaporation of the solvent is delayed sufficiently to enable it to attack the outer surfaces of the said grains of bituminous material, softening said surfaces and causing said grains to adhere and form a stiff plastic mass, and, third, in laying said plastic mass in the desired form or position before the action of the said solvent extends to and dissolves the interior parts of the said grains of bituminous material.

In testimony whereof I have signed my name to this specification in the presence of two subscribing witnesses.

HERBERT PASCHKE.

Witnesses:

ISAAC B. OWENS,  
JNO. M. RITTER.